

H. C. LEESEBERG.

METHOD OF TREATING PISTONS AND PISTON RINGS TO PREVENT DISTORTION IN USE.  
APPLICATION FILED APR. 18, 1921.

1,412,288.

Patented Apr. 11, 1922.

FIG. 1.



FIG. 2.



FIG. 3.



FIG. 4.



INVENTOR

Henry C. Leeberg,  
By Carrie Quaint Crampton  
Atty.

# UNITED STATES PATENT OFFICE.

HENRY C. LEESEBERG, OF FOSTORIA, OHIO.

## METHOD OF TREATING PISTONS AND PISTON RINGS TO PREVENT DISTORTION IN USE.

1,412,288.

Specification of Letters Patent. Patented Apr. 11, 1922.

Application filed April 18, 1921. Serial No. 462,390.

*To all whom it may concern:*

Be it known that I, HENRY C. LEESEBERG, a citizen of the United States, and a resident of Fostoria, county of Seneca, and State of Ohio, have made an Invention Appertaining to Methods of Treating Pistons and Piston Rings to Prevent Distortion in Use; and I do hereby declare the following to be a full, clear, and exact description of the invention, such as will enable others skilled in the art to which it appertains to make and use the same, reference being had to the accompanying drawings, and to the characters of reference marked thereon, which form a part of this specification.

This invention relates particularly to the manufacture of pistons and piston rings.

In the use of cast iron pistons and piston rings as heretofore manufactured, at least so far as I am aware, it is found that they are practically all subject to warping more or less, the amount of distortion depending largely on the shape of the article and the internal strains that are set up in the process of cooling, and also on the temperature of the motor in which used and the vibrations and jars to which subjected during a running of the motor, such warping or distortion of the piston or rings permitting leakage past the same, as well understood in the art. It is found that there is no great distortion in the castings if they are used in the rough, the warping action taking place after metal has been removed from the casting by machining the various surfaces. To remedy such warping of the castings it has been customary to allow them to age or set after a machining operation, which process may take six or eight months, depending almost entirely upon the size of the casting and the accuracy that is required of the part after it has been completed. Unless this is done the finished parts will change shape and size.

The primary object of my invention is to so treat pistons or piston rings during the manufacture thereof as to eliminate strains and irregularities therein and to prevent warping and distorting occurring during use, and also to very materially reduce the time required in manufacturing articles of this class and treating or aging them to overcome the warping tendencies. It has not been customary, however, with piston ring manufacturers to permit the castings to age after being machined, and therefore

the rings when used are subject to the warping and distorting tendency to a much greater extent than would be the case if allowed to stand and age as is done with other castings when accurate work is desired. It is therefore one of the purposes of my invention to provide a process of treating rings to eliminate warping and distorting tendencies therein by a method which is simple and rapid to perform and can be practiced by manufacturers where time is a material object.

The invention is fully described in the following specification and a preferred method of practicing the same in the manufacture of piston rings is illustrated in the accompanying drawings, in which,—

Fig. 1 illustrates a ring as it appears in the first step of the process. Fig. 2 shows the ring split. Fig. 3 illustrates the heat treating operations, and Fig. 4 the finished ring after the final machining operation.

In the manufacture of a piston ring by my method, it is subjected to five main steps or operations as follows:—

First. The cast iron rings after being cast in the usual way are machined preferably, though not necessarily, to give them a rough finish on their outer peripheries, a plurality of rings during such operation being usually mounted side by side on a mandrel.

Second. The next step in the operation consists in transversely slitting the rings to make them of the split type used in pistons. This operation and the first operation do not differ from the operations heretofore practiced in the manufacturing of piston rings.

Third. After the machining and splitting operations the rings are reciprocated or agitated in an oven at a temperature from 300 to 900° F. for about three hours and then permitted to cool in the oven and to lay for a day or so. The time of exposure to the heat may be lengthened without detriment to the process. In practice it is found preferable to subject the rings to a temperature of between 600 and 700° F., although this temperature may be varied considerably and very good results obtained, the intention being to heat the articles to a temperature which is considerably above that to which they will be subjected in use. In this heating operation the rings are loosely mounted on a holding member which is reciprocated within the oven during the heat treatment

so as to subject the rings as nearly as possible to the motions and jarring actions to which subjected during use in an engine. A means of accomplishing this is illustrated 5 crudely in Fig. 3 in which 1 designates an oven, 2 a ring carrying member suspended within the oven from a crank-shaft 3, the member being adapted to have a plurality of rings loosely mounted thereon whereby a 10 turning of the shaft will impart a reciprocating movement to the member and rings.

Fourth. The next step in the process is to reheat the rings for about three hours at a temperature of approximately 400° F., or at 15 about 50° above the temperature to which subjected when in use, which in the ordinary motor usually runs between 300 and 350° F. The rings are then permitted to cool in the oven the same as before and to lay for a day 20 or so. The same oven as employed for the initial heating may be used and the rings subjected to the shaking or vibrating action during the heating.

Fifth. The final step in the operation is 25 to machine the rings in the usual or any suitable manner to correct any warping or irregularities remaining therein after the heating steps.

It is well known in the art that the tendency of cast iron to warp or set is greatly 30 increased after some of the metal has been removed therefrom by machining, and where accuracy is required castings must be aged or seasoned after each machining operation, 35 which process in each case takes from one to six months, depending on the size of the castings. I have found, however, that after subjecting the articles to the heat treatments as above described, they may be machined 40 repeatedly without causing any perceptible warping or distorting, and it is therefore apparent that my invention resides primarily in the heat treatment rather than in the machining operations, as the latter are 45 the same as performed with articles as now manufactured. In describing my method I have referred to the different machining steps with relation to the heating steps so that the invention might be fully understood. In practice the average piston ring 50 manufacturer does not pay much attention to the aging process for the reasons, first, that he usually is unable to get material fast enough and does not have time to allow it 55 to lay around for aging; and, second, the aging requires a great deal of extra space and work, and this means extra expense. With my process it is possible to accomplish in three days what, by the old method, would 60 require at least sixty days and be less certain in results.

While I have particularly described my process in connection with the manufacture of piston rings it will be understood that it 65 will be substantially the same for the manu-

facture of a piston, as a piston after receiving the initial machining operation would be subjected to the heating and reheating steps substantially as described in connection with the rings and reciprocated during such heat treatments, so that the piston during the heating would be subjected to approximately the same strains and vibrations as would be present when reciprocating in an engine. 70

After the heat treatments the piston is subjected to a final machining operation to correct any warping or irregularities therein. 75

Having thus described my invention, what I claim as new and desire to secure by Letters Patent, is,—

1. The method of treating cast iron pistons and piston rings to prevent warping and distorting in use, consisting in subjecting the articles for a period to a temperature above the temperature to which subjected in use, 85 then allowing to cool and later reheating the articles in a temperature greater than that to which subjected in use and allowing to cool and lay for a period preparatory to finishing to correct warping and irregularities therein. 90

2. The method of treating cast iron pistons and piston rings to prevent warping and distorting in use, consisting in subjecting the articles for a period to a temperature above the temperature to which subjected in use, agitating the articles while in such temperature, then allowing to cool and later reheating the articles for a period in a temperature greater than that to which subjected in use and allowing to cool and lay 100 for a period preparatory to finishing to correct warping and irregularities therein. 95

3. The method of treating cast iron pistons and piston rings to prevent warping and distorting in use, consisting in simultaneously reciprocating and heating the articles in a temperature above that to which the articles are subjected in use and then allowing to cool. 105

4. The method of treating cast iron pistons and piston rings to prevent warping and distorting in use, consisting in simultaneously reciprocating and heating the articles in a temperature above that to which the articles are subjected in use, then allowing to cool, and later simultaneously reciprocating and reheating the articles in a temperature above that to which subjected in use and allowing to cool. 110

5. The method of treating cast iron pistons and piston rings to prevent warping and distorting in use, consisting in subjecting the articles for a period to a temperature between 300° and 900° F. then allowing to cool and lay for a period, then reheating the articles in a temperature greater than the temperature to which subjected in use and then allowing to cool and lay for a period preparatory to finishing to correct warping and irregularities therein. 115

6. The method of treating cast iron pistons and piston rings to prevent warping and distorting in use, consisting in reciprocating the articles in an oven for about three 5 hours in a temperature above that to which subjected in use, then permitting to cool and to lay for a day or so, then reheating the articles for about three hours in a temperature above that to which the articles are subjected 10 in use, and then allowing to cool and lay for a day or so preparatory to finishing to correct warping and irregularities therein.

7. The method of treating cast iron pistons and piston rings to prevent warping and 15 distorting in use, consisting in reciprocating

the articles for about three hours in a temperature between 300° and 900° F. which temperature should be above the temperature to which the articles are subjected in use, allowing the articles to cool and to lay for 20 a period, then reheating the articles for a period in a temperature about 50° above the temperature to which subjected in use and allowing to cool and lay for a period preparatory to machine finishing to correct 25 warping and irregularities therein.

In testimony whereof, I have hereunto signed my name to this specification.

HENRY C. LEESEBERG.